

July 9, 1940.

C. H. COLEMAN

2,207,311

SPARK PLUG AND ELECTRODES THEREFOR

Filed Feb. 25, 1939



Inventor

*C.H. Coleman*

By *Watson E. Coleman*

Attorney

## UNITED STATES PATENT OFFICE

2,207,311

## SPARK PLUG AND ELECTRODES THEREFOR

Claude H. Coleman, Fairmead, Calif.

Application February 25, 1939, Serial No. 258,513

## 1 Claim. (Cl. 123—169)

This invention relates to improvements in igniting devices for internal combustion engines.

The present invention has for its primary object to provide an improved igniting device or spark plug in which the electrodes are made of commercially pure copper which has been hardened according to my improved process.

Another object of the invention is to provide an improved spark plug or internal combustion engine igniting device having hardened commercially pure copper electrodes which are secured in the device in such a manner that they may be replaced when, as and if necessary, so that the plug proper may be used indefinitely, the only repairs or replacements necessary being the occasional replacement of the electrodes thereof.

The invention will be best understood from a consideration of the following detailed description taken in connection with the accompanying drawing forming part of this specification, with the understanding, however, that the invention is not to be confined to any strict conformity with the showing of the drawing but may be changed or modified so long as such changes or modifications mark no material departure from the salient features of the invention as expressed in the appended claim.

The accompanying drawing illustrates a spark plug having electrodes formed of commercially pure copper hardened in accordance with my improved process and showing the manner in which such electrodes may be installed for easy replacement.

## In the drawing:

Fig. 1 illustrates a spark plug constructed in accordance with the present invention, the same being shown in side elevation.

Fig. 2 is a vertical longitudinal section through the same.

In setting forth the present invention, a description will first be given of the structure of the spark plug illustrated in the drawing after which a statement will be made of the process employed for hardening the copper from which the electrodes are made.

The numeral 1 generally designates the shell of the plug in which the upper portion is of polygonal contour, as indicated at 2, to facilitate the application of a wrench thereto whereby the threaded reduced lower end portion 3 may be secured in or unthreaded from the spark plug hole in the head of an internal combustion engine. Below the polygonal shaped portion 2 of the shell, the shell is provided with the encircling ribs or flanges 4 which serve to dissipate

heat by presenting an increased area of the body to the air.

The shell 1 is of the usual hollow form and is interiorly threaded at its upper end to receive a bushing 5 by means of which the insulation sleeve 6, of porcelain or other suitable insulation material, is maintained in position. This sleeve has the usual longitudinally extending passage therethrough, as indicated at 7, but this passage through a portion of its length at the lower end of the sleeve is of reduced diameter while at its upper end it is enlarged to receive the metal liner 8 which is interiorly threaded and in which is adapted to be engaged the hollow binding nut 9, the inner end portion of which is provided with a pocket 10 for the purpose hereinafter described. This nut is formed to have the usual wire connection of the ignition mechanism made therewith. A suitable thin copper washer may be interposed between the top edge of the liner 8 and the binding nut 9, as indicated at 11.

The lower portion of the insulation bushing or sleeve 6 has an enlarged waist which is clamped between the bottom of the shell and the bushing and in order to prevent leakage, suitable copper washers 12 and 13 are interposed between the sleeve and the bushing and shell, as shown.

The lower edge of the reduced portion 3 of the shell is provided with a longitudinally extending threaded bore and threadably secured in this bore is one end of the ground electrode 14. By this means, this electrode may be removed and a new one substituted when necessary. The numeral 15 designates the central electrode of the plug which, as shown, has a thin or reduced lower end portion 16 and a larger upper end portion 17, which portions respectively position in the reduced lower portion of the passage 7 of the insulation sleeve and in the larger upper portion thereof in the manner shown. The upper end of the electrode 15 is frictionally held in the pocket 10 of the binding nut, so that when this nut is released from the liner 8 and removed, the central electrode may also be withdrawn to be replaced by a new one.

The electrodes 14 and 15 are formed from commercially pure copper which has been hardened by the following process, which process does not involve either alloying or working the metal. The copper selected is of the purest commercial grade obtainable, such copper normally averaging 99.98% purity. The impurities therein consist of lead which approximates .015%; silver, aluminum and magnesium approximating .0001%; calcium and silica approximating .001%. These im-

purities were determined by spectrographic analysis, in a specimen selected for use in the present invention and for hardening as hereinafter described, the copper, constituting by difference, 5 99.98%.

In treating the selected copper according to the present process, the metal is first reduced in temperature to slightly below the freezing point of water or, in other words, to 32° F. or slightly 10 below, and after being reduced to such temperature, it is then immersed in a bath of beef tallow which has been heated to a temperature of approximately 240° F., the immersion being for a period of approximately 20 seconds more or less 15 according to the size or thickness of the piece of metal treated. Immediately following this step, the metal is transferred to a soap solution which is maintained at boiling point. This soap solution may be made from any suitable laundry or 20 other type of soap and has a density of approximately 1.009. The metal is allowed to remain in this boiling soap solution for approximately 30 seconds. Following this last step, the metal is removed and thoroughly dried and allowed to 25 come back to approximately room temperature or from between 60° and 80° F. It is then subjected to a second chilling step wherein the temperature is reduced to approximately 10° below zero. After this desired temperature reduction 30 has been obtained in the metal, it is again immersed in the hot tallow solution, the temperature of which has been raised to approximately 280° F. and allowed to remain approximately 20 seconds after which it is transferred to the boiling 35 soap solution for 30 seconds and is subsequently thoroughly dried and allowed to return to normal or room temperature preparatory to carrying out the third step of the operation. Repetition of the last described series of steps is 40 made as many times as may be desirable to bring about the desired hardness of the metal and with each repetition of the three steps of chilling, immersion in hot tallow and then in the soap solution, the temperature of the tallow is raised about 45 10°. The first rise is from 240° to 280° F. and after that, the 10° increases are made until the desired degree of hardness is attained. Following the second series of steps, the reduction in the temperature of the metal is not increased. 50 The metal is reduced each time to approximately 10° below zero, and the maximum temperature for the tallow is approximately 400° F.

It has been found that in the foregoing process, the reaction occurring in rapidly changing the metal from the chilled condition to a highly heated condition in hot tallow or in any other similar fluid by means of which the temperature can be rapidly raised out of contact with the air, has the effect of hardening and toughening the metal without permitting any oxidation to occur. 5

Commercially pure copper treated according to the above described process may be hardened to 10 a degree where it may be made into spark plug terminals which will stand the high degrees of heat occurring in an internal combustion engine cylinder. Such tempered or hardened copper is 15 also employed for making the shell and bushing portion of the plug and has been found to dissipate heat more rapidly than steel or other metals used for this purpose and thereby prevent over-heating of the points and preignition. 20

From the foregoing, it will be apparent that the spark plug structure, particularly described, is novel in the provision of means for removal and replacement of the electrodes and is also novel in the use of the hardened copper electrodes. The use of such electrodes will materially cheapen 25 the production cost of such plugs as the material for the same and the process of hardening the material is relatively inexpensive as compared with the metals at present used for electrode points. 30

What is claimed is:

A spark plug, comprising a shell, an insulation body supported in and extending through the shell, said insulation body having a passage extending longitudinally therethrough, a ground electrode secured to one end of the shell in spaced relation with said insulation body, an interiorly threaded collar secured in the insulation body at the end thereof remote from the ground electrode, a terminal body threadably secured in said 40 collar, a central electrode having an end secured to said terminal body and extending therefrom through the passage of the insulation body and terminating in close proximity to said ground electrode, said central electrode being designed to 45 be withdrawn through the collar supporting end of the insulation body with said terminal body, and said electrodes being formed of hardened high temperature resisting copper. 50

CLAUDE H. COLEMAN.